

## UNITED STATES PATENT OFFICE

2,199,458

## ELECTRIC CONTACT

Franz R. Hensel, Kenneth L. Emmert, and James W. Wiggs, Indianapolis, Ind., assignors to P. R. Mallory & Co., Inc., Indianapolis, Ind., a corporation of Delaware

No Drawing. Application August 15, 1939,  
Serial No. 290,222

4 Claims. (Cl. 200—166)

This invention relates to electric contacts.

An object of the invention is to improve the characteristics of silver base electric contacts.

Another object of the invention is to provide

5 a silver base contact material which is highly resistant to tarnishing, and therefore will not form a layer of high contact resistance.

A still further object is to provide a new contact material which can be used under severe electrical conditions without welding.

10 It is a further object of the invention to provide a contact capable of operating on high frequency at heavy current values, without objectionable contact metal transfer.

15 Other objects of the invention will be apparent from the following description, taken in connection with the appended claims.

The present invention comprises the combination of elements, methods of manufacture and the 20 product thereof, brought out and exemplified in the disclosure hereinafter set forth, the scope of the invention being indicated in the appended claims.

While a preferred embodiment of the invention is described herein, it is contemplated that considerable variation may be made in the method of procedure and the combination of elements, without departing from the spirit of the invention.

25 The present invention comprises an improvement in electrical contacts which contain silver as the preponderant metal by weight. According to the invention, the contacts are improved by the addition of metals of second group of the 30 periodic system of elements in the fourth, sixth, and eighth series, namely calcium, barium, and strontium.

Accordingly, the contacts may be binary compositions containing calcium, barium, and strontium in approximately the following proportions by weight:

|               | Per cent |
|---------------|----------|
| (1) Calcium   | .02 to 5 |
| Silver        | Balance  |
| (2) Barium    | .02 to 5 |
| Silver        | Balance  |
| (3) Strontium | .02 to 5 |
| Silver        | Balance  |

45 It is likewise possible to improve the characteristics of silver alloys containing additional ingredients, by the addition of calcium, barium or strontium, thus silver alloys containing beryllium, magnesium, zinc, cadmium, copper, gold, nickel, manganese, thorium, platinum group elements,

silicon, titanium, zirconium, tin, indium, can be improved by the addition of calcium, barium, or strontium, in substantially the proportions indicated above.

The calcium, barium or strontium are added 5 in proportions greater than are necessary as de-oxidizers alone, so that the indicated proportion of these elements is retained as part of the finished alloy. Hence, especially in cases where additional ingredients are added to the alloy it may 10 be necessary to initially add amounts of these elements somewhat higher than the amount desired and in these cases the added calcium, barium or strontium may be within the range .5 to 15 5% or 1 to 5%.

The silver content, where other contact metals are present, should preferably amount to not less than about 75%.

The alloys of the present invention may be cast into desirable shapes and forms for the manufacture of electrical contacts. They may be cold worked by swaging, drawing, or rolling in reductions not exceeding 5% in area per pass or a total reduction of not over 15% in area. The allowable reduction increases as the proportion 25 of added element is decreased.

It is entirely within the scope of this invention to employ ternary and quaternary alloys of silver containing any two or all three of the elements calcium, barium, and strontium up to 30 a total added percentage of 5% since we have found that the binary alloys of these metals with silver up to 5% by weight form eutectic systems similar in nature. Intermetallic compounds are formed in the binary systems which seem to be 35  $Ag_2Ba$ ,  $Ag_2Ca$ , and  $Ag_2Sr$ .

The metals calcium, barium and strontium have melting and boiling points as follows:

|               | Calcium     | Strontium   | Barium      | 40 |
|---------------|-------------|-------------|-------------|----|
| Melting point | ° C.<br>810 | ° C.<br>800 | ° C.<br>850 |    |
| Boiling point | 1,170       | 1,150       | 1,140       |    |

45 Accordingly, the metals have melting points which are 100°—160° C. below that of silver and boiling points in an intermediate range which is higher than the vaporization points of cadmium and zinc and about 1100°—1150° C. below the boiling point of fine silver.

Taking binary silver-calcium alloys as an example, test alloys were prepared by pressing calcium chips and shavings with silver powder to form high density discs which were used as mas- 55

r alloys. This method prevents undue oxidation of the calcium and facilitates high recovery of calcium when the melting is carried out in a reducing or neutral atmosphere. The alloy could be cast in pre-heated molds, and care must be taken to keep the pouring temperature, or a little below, 960° C. If the alloy is poured too hot, porosity of the casting results.

There is an additional advantage in using the above-mentioned pressed-disc master alloys. If the discs are present to high density, they will sink, or may be pushed, to the bottom of the melt and therefore form the desired alloy with a minimum of deterioration by oxidation. Calcium powder may be used in the preparation of the above described master alloy discs, in which case it is desirable to mix the calcium and silver powders in a nitrogen or other similar neutral atmosphere to prevent oxidation and absorption of moisture. Some hydrogen may be present in the mixing atmosphere, if desired.

In making silver-calcium alloys, the molten silver may be deoxidized before the silver-calcium master discs are added. If a deoxidant is to be used magnesium may be recommended for this purpose, particularly when the final alloy is to be used for electrical contacts, as in the present invention.

We found it unnecessary to use any deoxidizer in our work since all melting was carried out in an atmosphere of hydrogen. At temperatures below 700° C., pure hydrogen should not be kept in contact too long with high-calcium metal materials, for calcium hydride may be formed which is fairly stable up to approximately 675° C. This caution is particularly directed toward calcium metal powder and pressed powder materials containing calcium metal which has not been fully alloyed.

In a number of contact applications, silver is mixed with refractory materials, taken from the group of tungsten and molybdenum, or their compounds particularly carbides, and with metals taken from the iron group, such as nickel, cobalt and iron. These materials are prepared either by mixing the powders together, pressing them, and hot and cold working same into suitable forms from which contacts can be prepared by first pressing the refractory or iron group metals, and then impregnating same with a silver-calcium alloy. Since calcium is available in powder form, it can be readily incorporated into the powder mix, and during elevated temperatures, will alloy and diffuse into the silver resulting in a homogeneous alloy. Certain care is to be taken in producing these products, in order to avoid oxidation of the calcium as described above in connection with melting technique. Sintering in the presence of metallic calcium we have found to be an excellent protective method.

In the preceding paragraphs, various alloy-preparation methods have been described using calcium as an example. Since, as stated before, the addition metals of the present invention are similar in behavior, barium and strontium may be substituted wherever calcium is mentioned in the above description.

Using the methods described above, test alloys were prepared for contact investigations. The alloys were cast and cold-swaged into rod form. Contacts were machined from these rods for the tests described below.

These contact tests were made to compare the performance of fine silver contacts with the be-

havior of contacts containing 2.5% of calcium, barium and strontium in binary alloys, under identical conditions of voltage, current, type of lead, contact pressure and frequency of operation wherein the current was gradually increased at intervals of 4 minutes until failure by welding took place.

Taking silver plus 2.5% calcium as a typical example, it was found that the material would withstand a 25% heavier current lead than fine silver. Specifically, where fine silver contacts would fail by welding at 12 amperes, our new contact alloy would carry 15 amperes before failure took place. By increasing the proportion of calcium to 3% by weight, it was found that the limiting current was increased to 17 amperes, and the transfer was further decreased. Under the same conditions, binary silver alloys containing barium and strontium had limiting currents in the range of 13 to 16 amperes, depending upon the amount of addition metal present. Alloys of the present invention were investigated over the range set forth in the appended claims. These tests were made at 12 volts D. C. 150 grams contact pressure, and on resistive-inductive load consisting of a rheostat in series with a 0.1 milli-henry inductance.

The alloys containing 0.5% of addition metal maintained low contact resistance. This was investigated by operating the contacts 72,000 times at a frequency of 20 operations per minute on resistive load at values shown below:

| Voltage   | Current | Ave. contact resistance |           | 35 |
|-----------|---------|-------------------------|-----------|----|
|           |         | Amperes                 | Milliohms |    |
| 12 D. C.  | 3       |                         | 0.9       |    |
| 110 D. C. | 1       |                         | 2.0       |    |
| 18 A. C.  | 6       |                         | 1.5       |    |
| 110 A. C. | 7       |                         | 2.5       | 40 |

These values are accepted as low contact resistance in the art, especially at the contact pressure employed, which was 50 grams.

We have found that contact alloys of the present invention are useful in differential combinations with other contact materials on D. C. circuits. It is possible to employ our alloys to advantage for the negative (cathode) contact in conjunction with positive contacts made of other materials of different composition. For resistive loads, we may use positive contact alloys such as silver-copper nickel, silver-gold-nickel, silver-tungsten, etc. For inductive loads, it is advisable to use positive contact materials such as silver-cadmium, silver-cadmium-nickel, silver-gold-nickel, etc.

The improvement obtained by such use of the alloys containing calcium, strontium, or barium is an increase in limiting current with a decrease in transfer of material between contacts. The increased limiting current, we believe, is due to anti-wetting properties conferred on the contacts by the oxides of calcium, barium, or strontium. The decreased transfer is obtained by using a positive contact alloy which has low transfer tendency under the type of electrical load imposed on the contacts.

The alloys of the present invention have a very satisfactory hardness. As a matter of fact, values such as 90 to 95 Rockwell F, can be readily obtained. With such hardness values, the contacts will show not only good electrical erosion resistance, but also mechanical wear resistance. In many cases, these contacts are used for re-

lays where mechanical wear in the order of a very small fraction of an inch, will mean failure.

In cases where additional hardness is required to withstand mechanical wear, we have incor-

porated small amounts of copper and/or nickel into the above-described binary compositions. We have also added small amounts of cobalt or manganese for the same purpose. The percentage of nickel, cobalt or manganese is kept below 10%.

Copper may be added, however, to the extent of 10%. These materials act to restrain grain growth and to inhibit softening at high temperatures.

The alloys were also tested for tarnish resistance by placing same in a chamber through which hydrogen sulphide was passed. For comparison, fine silver and some of the standard silver alloys were tested. It was found that while fine silver would show a very heavy sulphide coat, within a period of 24 hours, the alloys of the present invention maintained a bright surface for the same length of time, and showed only a slight tarnish film at the end of 72 hours. When testing the contact resistance, it was found that the improved alloys of the present invention showed contact resistance values of the same order, after the sulphiding test, as were obtained before sulphiding.

The present alloy has been found particularly useful for such applications as sensitive relays, thermostatic control contacts, overload relay contacts, differential contacts in general, etc.

Because of their lower specific gravity and decreased proportion of silver, alloys of the present invention are lower in cost per given contact shape, than contacts fabricated from fine silver.

While the present invention as to its objects and advantages has been described herein as carried out in specified embodiments there-

of, it is not desired to be limited thereby, but it is intended to cover the invention broadly within the spirit and scope of the appended claims.

What is claimed is:

1. An electric contact element formed of an alloy comprising .02 to 5% of material selected from the group of elements consisting of calcium, barium and strontium as an essential alloying ingredient, and the balance predominantly silver. 10

2. An electric contact element formed of an alloy comprising .02 to 5% of material selected from the group of elements consisting of calcium, barium and strontium as an essential alloying ingredient, and the balance predominantly silver, the silver content of said alloy amounting to not less than about 75%. 15

3. An electric contact formed of a heterogeneous bonded metal composition of finely divided refractory material selected from the group consisting of tungsten and molybdenum and their refractory compounds interspersed with and bonded by an alloy of .02 to 5% of material selected from the group of elements consisting of calcium, barium and strontium as an essential alloying ingredient and the balance substantially all silver. 20

4. An electric contact material formed of a heterogeneous bonded metal composition of finely divided metal selected from the group consisting of nickel, cobalt and iron interspersed with and bonded by an alloy of .02 to 5% of material selected from the group of elements consisting of calcium, barium and strontium as an essential alloying ingredient and the balance predominantly silver. 35

FRANZ R. HENSEL.  
KENNETH L. EMMERT.  
JAMES W. WIGGS.